



ing has been finished immediately before coating. Furthermore, the novel surface active agent of this invention, if desired, may be used together with other conventional surface active agents.

The optimum amount of the amphoteric surface active agent is varied in accordance with various conditions, such as the type of coating composition, the manner of coating and the like, but in general the addition of 0.01-0.2% by weight of the surface active agent based on the weight of the coating composition gives the best effect. This amount corresponds to 0.1-2.0 g. per one kg. of gelatin in the coating composition.

According to the process of this invention, a photographic emulsion containing the aforesaid surface active agent can be uniformly applied to a support with a high speed without deleterious effect on the photographic properties of the light-sensitive element. In particular, after developing the color photographic light-sensitive element containing the surface active agent of this invention, color images having good fastness can be obtained.

Furthermore, since the amphoteric surface active agent used in this invention causes few undesirable reactions with other additives of the emulsion, difficulties otherwise encountered during production of photographic light-sensitive elements are reduced.

The invention will now be explained in detail by reference to the following examples, in which compounds I-IV are the surface active agents of the present invention, while compound V stands for a conventional surface active agent shown by the aforesaid general Formula A in which R is  $C_{14}H_{29}$ , R' is  $C_2H_4$ ; and  $p+q$  is 5.

#### Example 1

An emulsifier dispersion prepared by dispersing a solution of 2.3 g. of a cyan coupler having the following formula:



in 5.0 ml. of tri-ortho-cresylphosphate ester in 40 ml. of an aqueous 10% gelatin solution containing 0.2 g. of sodium n-dodecylbenzene sulfonate was added to 100 g. of a red-sensitive photographic emulsion containing 7 g. of gelatin and 5 g. of silver chlorobromide.

Into each of such emulsions were added 5 ml. of a 1% solution of compound I, II, III, IV or V and 3 ml. of a 3% acetone solution of triethylene phosphorous amide as a hardening agent, and the coating composition thus prepared was applied to a triacetyl cellulose support followed by drying to provide a light-sensitive film. The light-sensitive film was red-exposed stepwise, developed in a color developer containing 4-amino-3-methyl-N, N-dimethylaniline hydrochloride as a developing agent and then subjected to subsequent processings, such as, bleaching, fixing, water-washing and drying, as in any conventional manner, to provide a colored sample. The colored samples thus obtained were subjected to the following fading tests: (A) the sample was maintained for 20 days under the conditions of 60° C. and 75% relative humidity; and (B) the sample was maintained for four hours at 120° C. The results are shown in the following table in which the initial optical density of the cyan-colored image was 2.0.

| Surfactant               | Fading percent in Test A | Fading percent in Test B |
|--------------------------|--------------------------|--------------------------|
| None (control)           | 3.0                      | 24                       |
| Compound I               | 2.7                      | 25                       |
| Compound II              | 2.5                      | 21                       |
| Compound III             | 3.4                      | 26                       |
| Compound IV              | 3.2                      | 23                       |
| Compound V (comparative) | 7.2                      | 55                       |

From the results, it was confirmed that by the incorporation of the conventional surface active agent V, the fading of the colored image was accelerated remarkably but no such marked acceleration of fading was observed in the case of incorporating the surface active agents I, II, III and IV of this invention. Also, by the addition of the surface active agent of this invention, fastness of the colored image similar to or higher than that of the control sample, in which no surface active agent was added, was obtained.

#### Example 2

Into a red-sensitive emulsion containing the coupler as shown in Example 1 were added 2.0 ml. of a 1% solution of each of Compounds I, II, III, and V, and 2.0 ml. of a 1% solution of a surface active agent having the following formula



The coating composition thus prepared was applied to a triacetyl cellulose film at 35° C. and set at 5° C. To the thus coated wet emulsion layer a coating composition prepared by adding 2 ml. of a 1% solution of a surface active agent, n-dodecylbenzene sulfonate, to 100 g. of a 2% gelatin solution was applied with various coating speeds. When the coating speed was increased over a definite speed, it became impossible to spread the second coating composition on the surface of the first emulsion layer. However, the upper limit of the coating speed was remarkably improved by adding compound I, II or III of this invention to the second coating composition, as shown in the following table.

| Surfactant:              | Limit of coating speed (m./min.) |
|--------------------------|----------------------------------|
| None (control)           | 9                                |
| Compound I               | 50                               |
| Compound II              | >55                              |
| Compound III             | 50                               |
| Compound V (comparative) | 42                               |

#### Example 3

Into 10 ml. of a 7% gelatin solution was added 3.3 g. of the emulsified dispersion of the coupler as in Example 1, and to the mixture was added 5 ml. or 10 ml. of a 1% solution of compound II, IV or V. The resulting mixture was allowed to stand for 6 hours or 12 hours at 40° C. and thereafter applied to a glass plate in a dry thickness of 25 microns followed by drying. Thereafter, the turbidity of the layer thus formed was measured, the results of which are shown in the following table:

| Surfactant     | Amount, ml. | Turbidity (relative value) |        |         |
|----------------|-------------|----------------------------|--------|---------|
|                |             | 0                          | 6 hrs. | 12 hrs. |
| None (control) |             | 8.2                        | 8.6    | 9.6     |
| Compound II    | 5           | 10.2                       | 10.2   | 13.0    |
| Do.            | 10          | 10.2                       | 11.7   | 13.7    |
| Compound IV    | 5           | 8.0                        | 9.2    | 12.0    |
| Do.            | 10          | 17.9                       | 18.3   | 18.9    |
| Compound V     | 5           | 11.2                       | 12.8   | 14.1    |
| Do.            | 10          | 20.1                       | 21.5   | 24.6    |

As is clear from the above results, by the addition of compounds II and IV of this invention, the colloidal stability of the coupler-containing the emulsified dispersion was significantly better than the conventional compound V. Further, the emulsion layer formed by the present invention has good transparency.

#### Example 4

An emulsified dispersion prepared by dispersing a solution of 2.0 g. of a yellow coupler having the formula:



in a 2.0 ml. of di-n-butylphthalic acid ester in 30 ml. of an aqueous 10% gelatin solution containing 0.2 g. of sodium n-dodecylbenzene sulfonate was added to 100 g. of a red-sensitive photographic emulsion containing 6 g. of gelatin and 6 g. of silver iodobromide.

Each of the emulsion samples thus prepared was mixed with 5 ml. of a 1% solution of compound I, II or V and 3 ml. of a 3% acetate solution of triethylene phosphorous amide, and the mixture was applied to a triacetyl cellulose film followed by drying to provide a light-sensitive film. The light-sensitive film was then blue-exposed step-wise and processed as in Example 1 to provide a yellow image. The blue density  $D_b$  and red density  $D_r$  of the image were measured, the results of which are shown in the following table. The blue density  $D_b$  shows the relative strength of yellow coupling and the red density  $D_r$  shows the relative density of a silver image remaining after processing.

| Surfactant       | $D_b$ | $D_r$ |
|------------------|-------|-------|
| Compound I.....  | 2.0   | 0.07  |
| Compound II..... | 2.0   | 0.05  |
| Compound V.....  | 2.0   | 0.35  |

As shown in the results, when using compounds I and II of this invention, the silver image was removed effectively by bleaching and clear yellow dye images were obtained whereas when using the conventional compound V, silver images remained to a considerable extent.

What is claimed is:

1. A photographic coating composition comprising a gelatin containing silver halide emulsion and a minor amount of a surface active agent having the formula:



wherein R is an alkyl group having 8-20 carbon atoms and p and q each represent positive integers.

2. The composition of claim 1 wherein R is  $\text{C}_{12}\text{H}_{25}$  and  $p+q$  is 2.

3. The composition of claim 1 wherein R is  $\text{C}_{14}\text{H}_{29}$  and  $p+q$  is 2.

4. The composition of claim 1 wherein R is  $\text{C}_{14}\text{H}_{29}$  and  $p+q$  is 5.

5. The composition of claim 1 wherein R is  $\text{C}_{14}\text{H}_{29}$  and  $p+q$  is 30.

6. The composition of claim 1 wherein said surface ac-

tive agent is present in an amount of 0.01-0.2% by weight based on the weight of the coating composition.

7. The composition of claim 1 wherein said silver halide emulsion contains a suitable coupling agent.

8. The composition of claim 1 wherein said silver halide is silver chlorobromide.

9. The composition of claim 1 wherein said silver halide is silver iodobromide.

10. The composition of claim 7 wherein said coupling agent is a cyan coupler having the formula:



11. A photographic element comprising a support having applied thereto a photographic coating composition comprising a gelatin containing silver halide emulsion and a minor amount of a surface active agent having the formula:



wherein R is an alkyl group having 8-20 carbon atoms and p and q of each represent positive integers.

12. The element as claimed in claim 11 wherein R is  $\text{C}_{12}\text{H}_{25}$  and  $p+q$  is 2.

13. The element as claimed in claim 11 wherein R is  $\text{C}_{14}\text{H}_{29}$  and  $p+q$  is 2.

14. The element as claimed in claim 11 wherein R is  $\text{C}_{14}\text{H}_{29}$  and  $p+q$  is 5.

15. The element as claimed in claim 11 wherein R is  $\text{C}_{14}\text{H}_{29}$  and  $p+q$  is 30.

16. The element as claimed in claim 11 wherein the amount of said compound is 0.01-0.2% by weight of the coating composition.

#### References Cited

#### UNITED STATES PATENTS

45 3,441,413 4/1969 Nishio et al. ----- 96-114.5

NORMAN G. TORCHIN, Primary Examiner

J. R. HIGHTOWER, Assistant Examiner